

## 1

3,331,701

OIL REPELLENT COMPOSITIONS, METHODS FOR  
MAKING SAME AND TEXTILES TREATED  
THEREWITH

Domenick Donald Gagliardi, East Greenwich, R.I., assignor to Colgate-Palmolive Company, New York, N.Y., a corporation of Delaware  
No Drawing. Filed Sept. 30, 1963, Ser. No. 312,296  
20 Claims. (Cl. 117—121)

The present invention relates to the preparation of water-, oil-, and soil-repellent hydrophilic oxides and to textiles, including fibers, yarns, woven materials, felted materials, and leather treated therewith. More particularly, the present invention relates to the treatment of cationic oxides, water-insoluble inorganic oxides such as alumina, titania, zirconia, silica, zinc oxide and the like to provide treated oxide which is resistant to wetting by water, water-borne stains, oil, oil-borne stains, and to soiling by oily treated with the aforesaid cationic oxides to impart to said particulate soil and to fibrous materials, e.g., textiles treated with the aforesaid cationic oxides to impart to said fibrous materials the capability of resisting wetting by water and/or oil.

It has been known to coat regenerated cellulose products and more particularly filaments and staple fibers of viscose rayon to deposit thereon finely divided silica to improve the resistance of the fiber to soiling. However, the deposited silica, particularly that deposited on the outer surface of the fiber and not in the fiber crevices, has a tendency to become disassociated from the fiber during opening, carding, drawing and other such mechanical operations in which the coated fibers rub one against the other. In U.S. Patent No. 2,983,625 an improvement is disclosed wherein the fiber containing the silica deposited thereon is treated with alkylene oxide products of polyhydroxy alcohol esters of higher fatty acids whereby the fiber is substantially improved with respect to carding, drafting, softness, and "hand" or feel and the amount of silica retention without dusting for any particular method of depositing the silica on the fiber is substantially increased.

In U.S. Patent No. 3,031,335 there is disclosed a method of producing oil- and water-resistant fabrics in a two-step process involving immersion of the fabric in a solution of a salt such as aluminum acetate, zirconium nitrate, zirconium butoxide, drying the fabric, and immersing the dried fabric in a solution of perfluoromonocarboxylic acid, such as perfluoroctanoic acid, perfluorodecanoic acid, or one of the salts thereof. As illustrated the finished fiber consists of the fiber core, a layer of the aluminum or zirconium salt, and superposed thereon a second layer of the perfluoromonocarboxylic acid or salt.

In distinct contrast to the aforescribed product, the product of the present invention is a water- and oil-repellent as well as soil-repellent fiber or textile which in its simplest form consists of a core of fibrous material and a single layer of the treated cationic inorganic oxide.

In general, a water-soluble cationic oxide such as alumina, titania, zirconia, silica, zinc oxide, or mixtures of such water-insoluble cationic oxides, for example, bentonites, clays and the like in finely divided state is reacted with at least one fluorinated aliphatic monocarboxyl-

## 2

ic acid having four to twenty-two carbon atoms in which at least 70 percent to 100 percent of the non-carbon-to-carbon valences of the non-carboxylic carbon atoms is attached to fluorine atoms and has at least two and preferably three fluorine atoms attached to the terminal or omega carbon atom. In general, the perfluoroalkylmonocarboxylic acids have a composition corresponding to the formula:



10 where X is  $CHF_2$  or  $CF_3$ ; n is 3 to 20 and percent F=at least 70%  $[X+(CH_2)_n]$ .

Thus, for example fifty parts by weight of finely divided aluminum oxide were mixed with five hundred parts by weight of isopropanol (a solvent for the perfluoro aliphatic monocarboxylic acid) and four parts by weight of pentadecafluoroctanoic acid (perfluoroctanoic acid). The reaction mixture was refluxed at 82.5° C. for one hour and cooled to room temperature. The cooled reaction mixture was filtered, the white filter cake was washed with alcohol and dried. Gravimetric analysis established that the aluminum oxide had combined with about 5.6 percent of the perfluoroctanoic acid based upon the weight of aluminum oxide used.

Illustrative of the preparation of the treated cationic inorganic oxide and a method of applying the reaction product to textile material is the treatment of alumina with pentadecafluoroctanoic acid and the padding of cotton with the reaction dispersion. Alumina was reacted with pentadecafluoroctanoic acid in isopropanol in the ratios of 1:1, 10:1, 100:1, and 1,000:1 by weight at reflux temperature (about 82° C.) for about one hour. The reaction mixtures were cooled and 80 x 80 cotton padded with the cooled dispersions to 80 percent wet pick-up. The treated cotton was dried 24 hours at room temperature. The so-treated cotton and untreated cotton were subjected to the "Oily Particulate Soil Repellency" test described hereinafter with the results set forth in Table I.

TABLE I

| Ratio, Alumina to PDFA | Percent B | Reflectance A |
|------------------------|-----------|---------------|
| Untreated Cotton.....  | 26        | 77            |
| 3% of 1:1.....         | 50        | 78            |
| 3% of 10:1.....        | 42        | 76            |
| 3% of 100:1.....       | 57        | 76            |
| 3% of 1,000:1.....     | 58        | 76            |

The data presented in Table I make it manifest that the treated cotton sheds oily particulate soil.

Alternatively, the reaction product, i.e., the perfluoroacid treated cationic oxide is separated from the reaction mixture, washed with a solvent for the perfluoroacid, suspended in water with or without a surfactant and the textile padded or otherwise treated with the aqueous dispersion.

50 The water and oil repellency properties of alumina particles treated with various perfluoromonocarboxylic acids are shown in Table I. The original alumina particles had a water and oil repellency rating of zero.

55 Illustrative of the water- and oil-repellency properties conferred on cationic water-insoluble inorganic oxides per se by treatment with perfluoromonocarboxylic acids are the data presented in Table II obtained from the treatment of alumina particles with various perfluoro-

monocarboxylic acids. The untreated particles of alumina had water- and oil-repellency rating of zero.

Rating:

Characterized by

80 --- Wetting of the upper surface at spray points.

TABLE II

| Weight Ratio of Alumina to Per-fluoro acid | Reaction Product Dried Down |      |                    |    | Reaction Mixture Filtered and Cake Dried |      |       |     | Reaction Mixture Filtered, Cake Washed with IPA, Filtered and Dried |       |       |       | Reaction Mixture Filtered, Cake Washed with Acetone, Filtered and Dried |       |       |       |
|--------------------------------------------|-----------------------------|------|--------------------|----|------------------------------------------|------|-------|-----|---------------------------------------------------------------------|-------|-------|-------|-------------------------------------------------------------------------|-------|-------|-------|
|                                            | Oil <sup>1</sup>            |      | Water <sup>2</sup> |    | Oil                                      |      | Water |     | Oil                                                                 |       | Water |       | Oil                                                                     |       | Water |       |
|                                            | NG                          | G    | NG                 | G  | NG                                       | G    | NG    | G   | NG                                                                  | G     | NG    | G     | NG                                                                      | G     | NG    | G     |
| 1:1PDFA                                    | 100+                        | 100+ | 0                  | 90 | 100+                                     | 100+ | 100   | 100 | 90                                                                  | 80    | 100   | 100   | 50                                                                      | 70    | 100   | 100   |
| 1:1PFB                                     | 80                          | 100  | 100                | 90 | 80                                       | 90   | 90    | 90  | -----                                                               | ----- | ----- | ----- | -----                                                                   | ----- | ----- | ----- |
| 1:1TFA                                     | 0                           | 0+   | 0                  | 0  | 0                                        | 0+   | 0     | 0   | -----                                                               | ----- | ----- | ----- | -----                                                                   | ----- | ----- | ----- |

<sup>1</sup> Same rating system as that of 3M oil-heptane test described hereinafter.

<sup>2</sup> Rating applying water drop to treated cloth with medicine dropper.

100—drop rolled off.

90—drop did not penetrate in three minutes.

Alumina and pentadecafluoroctanoic acid were reacted for about one hour at reflux temperature (about 80° C.) in isopropanol. The reaction product was padded on cotton (80 x 80) from isopropanol or water suspension and dried. The oil repellency and resistance to soiling with oily particulate soil were determined. The results are presented in Table III.

25

TABLE III

| Dispersion             | Cured at Room Temperature |             |    |
|------------------------|---------------------------|-------------|----|
|                        | Repellency Oil            | Reflectance |    |
|                        |                           | B           | A  |
| 1% in IPA              | 90                        | 43          | 77 |
| 1% in H <sub>2</sub> O | 90/80                     | 44          | 78 |
| 3% in IPA              | 100/90                    | 48          | 78 |
| 3% in H <sub>2</sub> O | 100/90                    | 50          | 78 |
| Untreated Control      | 0                         | 26          | 77 |

IPA—Isopropanol.

It will be observed that in every instance the treated cloth before washing had a higher reflectance than the untreated cloth. In other words, the treated cloth shed the oily particulate soil. Furthermore, it will be noted that treated cloth when cured at room temperature had excellent oil repellency.

It is manifest that controlled evaluating of fabric finishes in actual use is not possible. Consequently, it has been necessary to use evaluation methods subject to laboratory control which will simulate as closely as possible actual conditions under which water-repellency, oil-repellency, resistance to staining by water-borne and oil-borne stains, and resistance to staining by oily particulate soil of treated fabrics occurs. Such methods of evaluation are the following:

Water Repellency.—Resistance to wetting (spray test)  
AATCC Standard Test Method 22-1952

45

This test is applicable to any textile fabric. It measures the resistance of fabrics to wetting by a water spray and the results depend primarily on the degree of hydrophobicity inherent in the fibers and yarns and subsequent treatments to which the fabric is subjected. Water is sprayed against the taut surface of a test specimen. Evaluation of the wetted pattern is readily brought about by comparing the wetted pattern with standard wetting pattern pictures:

Rating: Characterized by

100 --- No sticking or wetting of the upper surface.  
90 --- Slight random sticking or wetting of the upper surface.

0—drop penetrated.

NG—not ground.

G—ground.

PDFA—pentadecafluoroctanoic acid.

PFB—perfluorobutyric acid, CF<sub>3</sub>(CF<sub>2</sub>)<sub>2</sub>COOH.

TFA—trifluoroacetic acid.

70 --- Partial wetting of the whole of the upper surface.

50 --- Complete wetting of the whole of the upper surface.

0 --- Complete wetting of the whole of the upper and the lower surfaces.

30 The test specimens of minimum size of 7" x 7" (seven inches by seven inches) are conditioned at 70° F. and 65 percent relative humidity for a minimum of four hours before testing.

35 The test specimen, fastened securely and wrinkle-free in a metal hoop having a diameter of 6 inches, is placed and centered 6 inches under a standard spray nozzle at an angle of 45° to the horizontal. Two hundred and fifty milliliters of water at 80±2° F. is poured into a funnel attached above the spray nozzle. The spray lasts 25 to 30 seconds at the end of which time the hoop is taken by one edge and the opposite edge tapped smartly once against a solid object with the wet side facing the solid; this procedure is repeated with the hoop reversed 180°.

40 Oil Repellency.—“3M Textile Chemicals” appendix  
A—test methods, page 1

45 The Minnesota Mining oil repellency test is based on the different penetrating properties of the two hydrocarbon liquids, mineral oil (“Nujol”) and n-heptane. (“Nujol” is the trade name for white mineral or paraffin oil being a mixture of hydrocarbons having a density for “light” oil in the range of 0.83 to 0.860 and for “heavy” oil in the range of 0.875 to 0.905.) The “Nujol”-heptane proportions for each rating were selected by “3M” to give oily stain resistance somewhat comparable to the water-borne stain resistance corresponding to each of the spray ratings of the AATCC Standard Test Method 22-1952.

| Oil Repellency Rating | Percent Heptane (by volume) | Percent “Nujol” (by volume) |
|-----------------------|-----------------------------|-----------------------------|
| 100+                  | 60                          | 40                          |
| 100                   | 50                          | 50                          |
| 90                    | 40                          | 60                          |
| 80                    | 30                          | 70                          |
| 70                    | 20                          | 80                          |
| 50                    | 0                           | 100                         |
| 0                     | -----                       | (1)                         |

1 No hold out to “Nujol.”

70 The standard oil-heptane mixtures are contained in small stoppered medicine-dropper bottles. A drop of each mixture of “Nujol” and heptane is placed on the fabric. The appearance of the test oil is observed through the drop. Note is made whether wetting or penetration occurs.

75 The number corresponding to that mixture containing the

highest percentage of heptane which does not penetrate or wet the fabric after three minutes is considered the oil repellency rating of the system.

The change in the optical refractivity of the drop is often an indication of wetting. In some cases wetting can be better determined by observing the other side of the fabric. In some cases reported hereinafter the term "0+" has been used to indicate a modicum of resistance to wetting by oil.

#### Stain repellency

The following procedures have been used to establish the degree of resistance to staining by water-borne and oil-borne stains of fabrics.

(a) The fabrics were stretched lightly on 12" x 31" frames. All or part of the frame was used depending upon the amount of fabric available. The frames were supported at both ends with the fabric about 8 inches above a black surface. The fabric touched nothing.

(b) Three inch medicine droppers were used to draw the stains from the containers. A 1 cubic centimeter calibration was established and marked on the exterior of each dropper. The stains were squeezed vertically downward from a height 2 inches above the cloth.

(c) After five minutes the unabsorbed stain was wiped off the fabric with two sweeps of "Kleenex" and the stains rated as follows:

| Appearance:             | Rating |
|-------------------------|--------|
| No stain visible        | 5      |
| Slight stain            | 4      |
| Easily noticeable stain | 3      |
| Considerable stain      | 2      |
| Very heavily stained    | 1      |

(The spread or lack of spread is not necessarily reflected in the ratings.)

(d) Duplicate sets of stains were applied in separate areas so that one-half of the fabric could be washed. In most instances, the wash was carried out with 50 grams of "FAB," a cotton cycle, and a dummy load to total 5 pounds in a Norge home automatic washer.

(e) The following two lists describe the numbering and the gross characterizations of the stains employed.

#### Water stains

1. Instant Tea a
2. Sheaffer's 232 Blue-black skrip
3. A&P Concord Grape Juice
4. "Ann Page" Salad Mustard
5. "Bosco" chocolate syrup

#### Oil stains

6. Wesson Oil
7. Gulf "Supreme" Motor Oil 20/20
8. Oleomargarine b
9. La Rosa Tomato Sauce
10. "Jergen's" Lotion

a 8 cc. dry powder/200 cc. water applied at 160° F.  
b Melted and applied at 160° F.

In reporting the relative resistance to staining and ease of stain removal in laundering, the staining values for water-borne and oil-borne stains were averaged separately.

In all cases the stains were allowed to dry on the fabrics for twenty-four hours before laundering.

#### Oily particulate soil repellency.—(GRC dry soil test)

Fifteen to twenty 6" x 8" numbered specimens (normally 80 x 80 cotton), including at least one untreated control, are tumbled for thirty minutes with 10 percent of "Cyanamid Soil" based on the weight of the fabric. The tumbling is carried out in a 5 liter capacity "Five Minute Home Cleaner" at 44 r.p.m.; six No. 8 neoprene rubber stoppers are distributed among the specimens to increase the mechanical action. At the end of tumbling, the specimens are removed and each shaken separately up and down fifteen times by hand to remove surface dirt.

The specimens are then cut in two (to produce two 4" x 6" pieces). One-half is washed with 50 grams of "FAB" in a cotton cycle with a 5-pound dummy load, then hung to dry and lightly ironed under a clean cotton cloth.

The degree of soiling is determined with a Photovolt Reflectance Meter (Tri Blue Filter). Six readings per specimen are made and the arithmetic average reported.

The "Cyanamid Soil" described below is the same as that recommended by Minnesota Mining and Manufacturing Co. The following dry ingredients are blended thoroughly, dried in a forced draft convection oven for eight hours at 50° C., then milled for twenty-five hours with ceramic balls and stored in a polyethylene bag.

#### "Cyanamid soil"

|    | Material                      | Percent by weight |
|----|-------------------------------|-------------------|
| 15 | Peat moss                     | 38                |
|    | Cement                        | 17                |
| 20 | Kaolin clay <sup>1</sup>      | 17                |
|    | Silica, 200 mesh <sup>2</sup> | 17                |
| 25 | Furnace black <sup>3</sup>    | 1.75              |
|    | Red iron oxide <sup>4</sup>   | 0.50              |
| 30 | Mineral oil                   | 8.75              |

<sup>1</sup> "Peerless" R. T. Vanderbilt.

<sup>2</sup> Davidson Chemical Co.

<sup>3</sup> "Molacco" Benny and Smith Co.

<sup>4</sup> C. K. Williams Co.

The aforescribed water-insoluble cationic inorganic oxides after treatment with perfluoromonocarboxylic acids are also useful for treating other substrates, e.g., ceramics, leather, paper, elastomer, e.g., natural rubber, synthetic elastomers and plastics to confer upon or impart thereto the capability of resisting soiling by oily particulate-soil. These treated water-insoluble cationic inorganic oxides can also be used as fillers for resins and elastomers including natural rubber.

What is claimed is:

1. A method of producing oil-repellent finishing agent for textiles which comprises heating a reaction mixture consisting essentially of from 1 to 1000 parts by weight of a finely divided water-insoluble, hydrophilic cationic inorganic oxide, per one part of perfluoroaliphatic monocarboxylic acid and solvent for said perfluoroaliphatic monocarboxylic acid at about the reflux temperature of said solvent, said perfluoroaliphatic monocarboxylic acid being an aliphatic monocarboxylic acid having four to twenty-two (inclusive) carbon atoms in the molecule of which at least seventy percent to one hundred percent of the non-carbon-to-carbon valences of the non-carboxylic carbon atoms is satisfied by fluorine atoms and at least two to three fluorine atoms are attached to the terminal carbon atom of the aliphatic chain of said monocarboxylic acid.
- 40 2. The method of producing oil-repellent finishing agent for textiles as set forth in claim 1 wherein the water-insoluble, hydrophilic, cationic inorganic oxide is alumina.
3. The method of producing oil-repellent finishing agent for textiles as set forth in claim 2 wherein the perfluoroaliphatic monocarboxylic acid is pentadecafluoroctanoic acid.
4. The method of producing oil-repellent finishing agent for textiles as set forth in claim 2 wherein the perfluoroaliphatic monocarboxylic acid is  $CF_3(CF_2)_2COOH$ .
5. The method set forth in claim 1 wherein the solvent is isopropanol.
- 65 6. A method of conferring oil-repellency as well as resistance to soiling with oily, particulate soil on textile material which comprises padding textile material to at least 70 percent wet pick-up in a suspension of water-insoluble, hydrophilic, cationic inorganic oxide treated with perfluoroaliphatic monocarboxylic acid, and curing said treated textile material at a temperature in the range of room temperature to 350° F. for a time inversely proportioned to the temperature and about five minutes at 300° F., said perfluoroaliphatic monocarboxylic acid having four to twenty-two carbon atoms in the molecule in

which at least 70 to 100 percent of the non-carbon-to-carbon valences of the noncarboxylic carbon atoms is satisfied by fluorine atoms.

7. The method of conferring oil-repellency as well as resistance to soiling with oily, particulate soil on textile material as set forth in claim 6 wherein the treated textile material is cured at room temperature.

8. The method of conferring oil-repellency as well as resistance to soiling with oily, particulate soil on textile material as set forth in claim 6 wherein the suspension of water-insoluble, hydrophilic, cationic inorganic oxide treated with perfluoroaliphatic monocarboxylic acid contains non-rewetting surfactant.

9. The method of conferring oil-repellency as well as resistance to soiling with oily, particulate soil on textile material as set forth in claim 6 wherein the suspension of water-insoluble, hydrophilic, cationic inorganic oxide treated with perfluoroaliphatic monocarboxylic acid contains at least one percent of said treated inorganic oxide.

10. The method set forth in claim 6 wherein the treated cationic inorganic oxide is suspended in isopropanol.

11. The method set forth in claim 6 wherein the treated cationic inorganic oxide is suspended in water.

12. A method of conferring oil-repellency as well as resistance to soiling with oily, particulate soil on textile material which comprises heating a reaction mixture comprising water-insoluble, hydrophilic, cationic inorganic oxide, perfluoroaliphatic monocarboxylic acid and solvent for said perfluoroaliphatic monocarboxylic acid at about the reflux temperature of said solvent, padding textile material to at least 70 percent wet pick-up in said reaction mixture, and curing the treated textile at a temperature in the range of room temperature to 350° F. for a time inversely proportioned to the temperature and about five minutes at 300° F., said perfluoroaliphatic monocarboxylic acid having four to twenty-two carbon atoms in the molecule of which at least seventy to one hundred percent of the non-carbon-to-carbon valences of the non-carboxylic carbon atoms is satisfied by fluorine atoms.

13. The method set forth in claim 12 wherein the solvent is isopropanol.

14. An oil repellent composition consisting essentially of the reaction product of 1 to 1000 parts by weight of a finely divided water-insoluble inorganic oxide with at least one part of perfluoroaliphatic monocarboxylic acid containing from 4 to 22 carbon atoms of which at least 70 percent to 100 percent of the non-carbon-to-carbon valences of the non-carboxylic carbon atoms is satisfied by fluorine atoms and at least 2 to 3 fluorine atoms are attached to the terminal carbon atom of the aliphatic chain of said non-carboxylic acid.

15. An oil repellent composition as defined in claim 14 wherein said inorganic oxide is alumina.

16. An oil repellent article comprising a fibrous material having affixed thereto as an oil repellent surface a composition as defined in claim 14.

17. An oil repellent composition as defined in claim 15 wherein the perfluoroaliphatic monocarboxylic acid is pentadecafluoroctanoic acid.

18. An oil repellent article as defined in claim 16 wherein the fibrous material is a textile material.

19. An oil repellent article as defined in claim 16 wherein the fibrous material is leather.

20. An oil repellent article as defined in claim 16 wherein the fibrous material is paper.

#### References Cited

##### UNITED STATES PATENTS

|    |           |         |              |           |
|----|-----------|---------|--------------|-----------|
| 30 | 2,547,042 | 4/1951  | Pole         | 117—118 X |
|    | 2,779,136 | 1/1957  | Hood et al.  | 117—118   |
|    | 2,953,474 | 9/1960  | Wheeler      | 117—100 X |
|    | 3,013,893 | 12/1961 | Olson et al. | 117—32 X  |
| 35 | 3,222,204 | 12/1965 | Weber et al. | 117—27    |

WILLIAM D. MARTIN, Primary Examiner.

MURRAY KATZ, Examiner.

40 T. G. DAVIS, Assistant Examiner.